

No. 773,524.

PATENTED OCT. 25, 1904.

W. S. ROGERS.  
COATED NAIL.

APPLICATION FILED MAR. 31, 1903.

NO MODEL.

*Fig. 1.*



*Fig. 2.*



WITNESSES

F. L. Ouraud.  
Weller & Dick

INVENTOR.

*William S. Rogers*  
*by*  
*Hannibal Dally*  
*Attorney.*

## UNITED STATES PATENT OFFICE.

WILLIAM S. ROGERS, OF CLEVELAND, OHIO, ASSIGNOR TO J. C. PEARSON COMPANY, OF BOSTON, MASSACHUSETTS, A CORPORATION OF MAINE.

## COATED NAIL.

SPECIFICATION forming part of Letters Patent No. 773,524, dated October 25, 1904.

Application filed March 31, 1903. Serial No. 150,356. (No model.)

*To all whom it may concern:*

Be it known that I, WILLIAM S. ROGERS, a citizen of the United States, and a resident of Cleveland, county of Cuyahoga, and State of Ohio, have invented a certain new and useful Improvement in Coated Nails, of which the following is a specification.

My process for the manufacture of coated nails is as follows:

10 Rosin is dissolved in gasoline or some readily-volatile solvent in about the proportion of thirty-two parts, by weight, of rosin to ninety-six parts, by weight, of gasoline, and a small quantity of a non-drying oil—such as fish-oil, 15 castor-oil, rosin-oil, or similar oil—is added to this solution in about the proportion of one part, by weight, of such oil to the above-given proportions of solution. It will be found that the above amounts of rosin and 20 fish-oil will be almost entirely dissolved in the above-named proportion of gasoline, especially if the mixture is allowed to stand for some time, although without the fish-oil the solution of the rosin would be far from complete. Other non-drying oils assist the solution in the same way in varying degrees, castor-oil being more effective in this respect than fish-oil, but is more expensive. Solution will take place at ordinary temperatures 25 without artificial heat. The nails to be coated are dipped in the cold solution, the surplus of which is then drained off from the nails, which are dried quickly by evaporating the gasoline or other volatile solvent, which does 30 not require heat.

By the use of this process a thin tough transparent practically-colorless coating of rosin and non-drying oil is left upon the nail or other article. On account of the presence 35 of the small amount of non-drying oil the coating is tough and not brittle and the nails so coated will not stick to each other. As the nails will not stick to each other, it is not necessary to break them apart when they have 40 dried or on removing them from the kegs in which they are packed, and there is no roughness or break in the coated surface, such as would be found if the surfaces were brittle and had stuck together and been separated,

as would often be necessary if the coating did not contain the non-drying oil.

The amount of the non-drying oil contained in the resinous solution is so small in proportion that it will not be unpleasantly perceptible to any extent in the handling or use 55 of the article, while it is sufficient to add toughness to the coating and prevent the coating from becoming brittle and flaky and to prevent the coated articles from sticking together after dipping and while they are dry- 60 ing and to increase the holding power of the nail when driven. A less amount even than that indicated will be sufficient for practical purposes, and if a very dry coating is wanted it is an advantage to add about one part, by 65 weight, of metallic resinate, such as lead resinate or manganese resinate, or both, to each one hundred parts of the non-drying oil. This is most conveniently done by adding the resinates to warm oil before the non-drying oil is 70 mixed with the rosin and gasoline.

The so-called "cement-coated" nails which have been for a long time sold in large quantities have a coating which softens by the heat and friction caused by driving the nail into 75 wood, and the coating is stripped from the nail and remains about the head of the nail near the surface of the first piece of wood penetrated. In consequence of this stripping of the coating from the cement-coated nails 80 now sold the greater part of the nail is not protected from moisture striking its sides, but only from moisture which might enter near the head of the nail, and the lower part of the nail often has no substantial coating 85 either to protect the nail from moisture or to adhere to the second piece of wood into which the nail is driven, whereby a large part of the value of the coating is lost.

The coated nails made in accordance with 90 this specification have a tough coating which will not strip off when the nail is driven into wood, although it will soften sufficiently by the heat developed in driving to make the nail very tenacious to the material into which 95 it is driven after the nail has been allowed to cool. The nail will be protected from moisture throughout its length, and the benefit of

the tenacity of the coating for the entire length of the nail is obtained. Another important feature is that the nail may be drawn from the wood and used again with its coating substantially intact, whereas the coated nails now used when withdrawn from the wood are substantially uncoated nails.

The process of making the composition without heat and applying it to the nails by 10 merely dipping the nails in the cold solution or pouring the cold solution over the nails and drying the coating by the mere evaporation of the gasolene at ordinary temperatures without artificial heat is a marked improvement over prior processes for coating nails. 15 Great care should be used, of course, to neglect none of the usual precautions to avoid an explosion of the gasolene.

The coated nails made by my process are 20 not only a great improvement on the coated nails now in the market as regards durability and tenacity, but they are very attractive in appearance, because their surfaces remain smooth and free from cracks and flakes during manufacture and sale. In fact, the coating is practically invisible.

Other substances may be added to the 25 rosin, non-drying oil, and the volatile solvent without departing from my invention, and 30 any readily-volatile solvent similar to gasolene

may be used, and I desire to be understood as including any such modification within my claim.

In the drawings accompanying this specification, Figure 1 represents a perspective of 35 the nail; Fig. 2, a section of the nail.

A represents the metal of the nail, and B the thin coating.

The drawings necessarily are largely diagrammatic. The coating B in the drawings 40 is opaque and of appreciable thickness; but in the actual nail it is a practically colorless and transparent film quite imperceptible to the eye.

What I claim as my invention is— 45

1. A coated nail coated with a composition consisting substantially of rosin and a proportionately small quantity of a non-drying oil, substantially as set forth.

2. A coated nail coated with a composition 50 consisting substantially of rosin and a proportionately small quantity of a non-drying oil, containing a small percentage of metallic resinate, substantially as set forth.

In testimony whereof I have hereunto set 55 my hand this 26th day of March, 1903.

WILLIAM S. ROGERS.

Witnesses:

CHAS. F. KROGG,  
FRED M. SAYLE.